



US008905147B2

(12) **United States Patent**  
**Frripp et al.**

(10) **Patent No.:** **US 8,905,147 B2**  
(b5) **Date of Patent:** **Dec. 9, 2014**

(54) **METHODS OF REMOVING A WELLBORE ISOLATION DEVICE USING GALVANIC CORROSION**

(75) Inventors: **Michael Frripp**, Carrollton, TX (US);  
**Syed Hamid**, Carrollton, TX (US); **Pete Dagenais**, Carrollton, TX (US)

(73) Assignee: **Halliburton Energy Services, Inc.**,  
Houston, TX (US)

(\*) Notice: Subject to any disclaimer, the term of this patent is extended or adjusted under 35 U.S.C. 154(b) by 370 days.

(21) Appl. No.: **13/491,995**

(22) Filed: **Jun. 8, 2012**

(65) **Prior Publication Data**

US 2013/0327540 A1 Dec. 12, 2013

(51) **Int. Cl.**  
**E21B 29/02** (2006.01)

(52) **U.S. Cl.**

USPC ..... **166/376**; 166/65.1; 166/317

(58) **Field of Classification Search**

CPC ..... E21B 29/00; E21B 29/02; E21B 34/063;  
E21B 34/14

USPC ..... 166/120, 317, 318, 376, 65.1

See application file for complete search history.

(56) **References Cited**

U.S. PATENT DOCUMENTS

7,350,582 B2 4/2008 McKeachnie et al.  
7,699,101 B2 4/2010 Frripp et al.

7,798,236 B2 9/2010 McKeachnie et al.  
8,211,248 B2 7/2012 Marya  
8,413,727 B2 4/2013 Holmes  
8,424,610 B2 4/2013 Newton et al.  
8,573,295 B2 11/2013 Johnson et al.  
2007/0181224 A1 8/2007 Marya et al.

(Continued)

FOREIGN PATENT DOCUMENTS

WO WO 2011017047 A1 2/2011  
WO WO 2013019409 A2 2/2013

OTHER PUBLICATIONS

Degradable Casing Perforation Ball Sealers and Methods for Use in Well Treatment, IPCOM000215741D, Mar. 7, 2012. Available at: <http://priorartdatabase.com/IPCOM/000215741>.

(Continued)

Primary Examiner — Jennifer H Gay

Assistant Examiner — Steven MacDonald

(74) Attorney, Agent, or Firm — John W. Wustenberg; Sheri Higgins Law; Sheri Higgins

(57) **ABSTRACT**

A wellbore isolation device comprises: at least a first material, wherein the first material: (A) is a metal or a metal alloy; and (B) is capable of at least partially dissolving when an electrically conductive path exists between the first material and a second material and at least a portion of the first and second materials are in contact with an electrolyte, wherein the second material: (i) is a metal or metal alloy; and (ii) has a greater anodic index than the first material. A method of removing the wellbore isolation device comprises: contacting or allowing the wellbore isolation device to come in contact with an electrolyte; and allowing at least a portion of the first material to dissolve.

**21 Claims, 2 Drawing Sheets**



(56)

**References Cited**

## U.S. PATENT DOCUMENTS

2008/0066924 A1 3/2008 Xu  
2008/0249637 A1\* 10/2008 Asgari ..... 623/23.72  
2010/0270031 A1\* 10/2010 Patel ..... 166/376  
2010/0294510 A1\* 11/2010 Holmes ..... 166/376  
2011/0132621 A1\* 6/2011 Agrawal et al. ..... 166/376  
2011/0136707 A1\* 6/2011 Xu et al. ..... 507/270  
2012/0118583 A1 5/2012 Johnson et al.  
2012/0175109 A1\* 7/2012 Richard ..... 166/250.12  
2012/0318513 A1 12/2012 Mazyar et al.  
2013/0032357 A1 2/2013 Mazyar et al.  
2013/0133897 A1 5/2013 Baihly et al.  
2013/0146302 A1\* 6/2013 Gaudette et al. ..... 166/376

2013/0206425 A1\* 8/2013 Mazyar et al. ..... 166/376  
2013/0327540 A1 12/2013 Hamid et al.  
2014/0027128 A1 1/2014 Johnson et al.

## OTHER PUBLICATIONS

Solu-Plugs—Delayed Frac Plugs, IPCOM000176055D, Nov. 3, 2008. Available at: <http://www.ip.com/pubview/IPC000176055D>.

T.Tanski, Synergy effect of heat and surface treatment on properties of the Mg—Al—Zn cast alloys, Journal of Achievements in Materials and Manufacturing Engineering, Oct. 2012, p. 260-274, vol. 54, Issue 2, Silesian University of Technology, Gliwice, Poland.

\* cited by examiner



FIG. 1



FIG.2



FIG.3



FIG.4

## METHODS OF REMOVING A WELLBORE ISOLATION DEVICE USING GALVANIC CORROSION

### TECHNICAL FIELD

An isolation device and methods of removing the isolation device are provided. The isolation device includes at least a first material that is capable of dissolving via galvanic corrosion when an electrically conductive path exists between the first material and a different metal or metal alloy in the presence of an electrolyte. According to an embodiment, the isolation device is used in an oil or gas well operation. Several factors can be adjusted to control the rate of dissolution of the first material in a desired amount of time.

### SUMMARY

According to an embodiment, a wellbore isolation device comprises: at least a first material, wherein the first material: (A) is a metal or a metal alloy; and (B) is capable of at least partially dissolving when an electrically conductive path exists between the first material and a second material and at least a portion of the first and second materials are in contact with an electrolyte, wherein the second material: (i) is a metal or metal alloy; and (ii) has a greater anodic index than the first material.

According to another embodiment, a method of removing a wellbore isolation device comprises: contacting or allowing the wellbore isolation device to come in contact with an electrolyte; and allowing at least a portion of the first material to dissolve.

### BRIEF DESCRIPTION OF THE FIGURES

The features and advantages of certain embodiments will be more readily appreciated when considered in conjunction with the accompanying figures. The figures are not to be construed as limiting any of the preferred embodiments.

FIG. 1 depicts a well system containing more than one isolation device.

FIGS. 2-4 depict an isolation device according to different embodiments.

### DETAILED DESCRIPTION

As used herein, the words "comprise," "have," "include," and all grammatical variations thereof are each intended to have an open, non-limiting meaning that does not exclude additional elements or steps.

It should be understood that, as used herein, "first," "second," "third," etc., are arbitrarily assigned and are merely intended to differentiate between two or more materials, etc., as the case may be, and does not indicate any particular orientation or sequence. Furthermore, it is to be understood that the mere use of the term "first" does not require that there be any "second," and the mere use of the term "second" does not require that there be any "third," etc.

As used herein, a "fluid" is a substance having a continuous phase that tends to flow and to conform to the outline of its container when the substance is tested at a temperature of 71° F. (22° C.) and a pressure of one atmosphere "atm" (0.1 megapascals "MPa"). A fluid can be a liquid or gas.

Oil and gas hydrocarbons are naturally occurring in some subterranean formations. A subterranean formation containing oil or gas is sometimes referred to as a reservoir. A reservoir may be located under land or off shore. Reservoirs are

typically located in the range of a few hundred feet (shallow reservoirs) to a few tens of thousands of feet (ultra-deep reservoirs). In order to produce oil or gas, a wellbore is drilled into a reservoir or adjacent to a reservoir.

5 A well can include, without limitation, an oil, gas, or water production well, or an injection well. As used herein, a "well" includes at least one wellbore. A wellbore can include vertical, inclined, and horizontal portions, and it can be straight, curved, or branched. As used herein, the term "wellbore" 10 includes any cased, and any uncased, open-hole portion of the wellbore. A near-wellbore region is the subterranean material and rock of the subterranean formation surrounding the wellbore. As used herein, a "well" also includes the near-wellbore region. The near-wellbore region is generally considered to 15 be the region within approximately 100 feet radially of the wellbore. As used herein, "into a well" means and includes into any portion of the well, including into the wellbore or into the near-wellbore region via the wellbore.

A portion of a wellbore may be an open hole or cased hole. 20 In an open-hole wellbore portion, a tubing string may be placed into the wellbore. The tubing string allows fluids to be introduced into or flowed from a remote portion of the wellbore. In a cased-hole wellbore portion, a casing is placed into the wellbore that can also contain a tubing string. A wellbore 25 can contain an annulus. Examples of an annulus include, but are not limited to: the space between the wellbore and the outside of a tubing string in an open-hole wellbore; the space between the wellbore and the outside of a casing in a cased-hole wellbore; and the space between the inside of a casing and the outside of a tubing string in a cased-hole wellbore.

It is not uncommon for a wellbore to extend several hundreds of feet or several thousands of feet into a subterranean formation. The subterranean formation can have different zones. A zone is an interval of rock differentiated from surrounding rocks on the basis of its fossil content or other features, such as faults or fractures. For example, one zone 35 can have a higher permeability compared to another zone. It is often desirable to treat one or more locations within multiples zones of a formation. One or more zones of the formation can be isolated within the wellbore via the use of an isolation device. An isolation device can be used for zonal isolation and functions to block fluid flow within a tubular, such as a tubing string, or within an annulus. The blockage of fluid flow prevents the fluid from flowing across the isolation 40 device in any direction and isolates the zone of interest. As used herein, the relative term "downstream" means at a location further away from a wellhead. In this manner, treatment techniques can be performed within the zone of interest.

Common isolation devices include, but are not limited to, a 45 ball and a seat, a bridge plug, a packer, a plug, and wiper plug. It is to be understood that reference to a "ball" is not meant to limit the geometric shape of the ball to spherical, but rather is meant to include any device that is capable of engaging with a seat. A "ball" can be spherical in shape, but can also be a 50 dart, a bar, or any other shape. Zonal isolation can be accomplished via a ball and seat by dropping the ball from the wellhead onto the seat that is located within the wellbore. The ball engages with the seat, and the seal created by this engagement prevents fluid communication into other zones downstream of the ball and seat. In order to treat more than one zone using a ball and seat, the wellbore can contain more than one ball seat. For example, a seat can be located within each zone. Generally, the inner diameter (I.D.) of the tubing string 55 where the ball seats are located is different for each zone. For example, the I.D. of the tubing string sequentially decreases at each zone, moving from the wellhead to the bottom of the well. In this manner, a smaller ball is first dropped into a first

zone that is the farthest downstream; that zone is treated; a slightly larger ball is then dropped into another zone that is located upstream of the first zone; that zone is then treated; and the process continues in this fashion—moving upstream along the wellbore—until all the desired zones have been treated. As used herein, the relative term “upstream” means at a location closer to the wellhead.

A bridge plug is composed primarily of slips, a plug mandrel, and a rubber sealing element. A bridge plug can be introduced into a wellbore and the sealing element can be caused to block fluid flow into downstream zones. A packer generally consists of a sealing device, a holding or setting device, and an inside passage for fluids. A packer can be used to block fluid flow through the annulus located between the outside of a tubular and the wall of the wellbore or inside of a casing.

Isolation devices can be classified as permanent or retrievable. While permanent isolation devices are generally designed to remain in the wellbore after use, retrievable devices are capable of being removed after use. It is often desirable to use a retrievable isolation device in order to restore fluid communication between one or more zones. Traditionally, isolation devices are retrieved by inserting a retrieval tool into the wellbore, wherein the retrieval tool engages with the isolation device, attaches to the isolation device, and the isolation device is then removed from the wellbore. Another way to remove an isolation device from the wellbore is to mill at least a portion of the device or the entire device. Yet, another way to remove an isolation device is to contact the device with a solvent, such as an acid, thus dissolving all or a portion of the device.

However, some of the disadvantages to using traditional methods to remove a retrievable isolation device include: it can be difficult and time consuming to use a retrieval tool; milling can be time consuming and costly; and premature dissolution of the isolation device can occur. For example, premature dissolution can occur if acidic fluids are used in the well prior to the time at which it is desired to dissolve the isolation device.

A novel method of removing an isolation device includes using galvanic corrosion to dissolve at least a portion of the isolation device. The rate of corrosion can be adjusted by selecting the materials used, the electrolyte used, and the concentration of free ions available in the electrolyte.

Galvanic corrosion occurs when two different metals or metal alloys are in electrical connectivity with each other and both are in contact with an electrolyte. As used herein, the phrase “electrical connectivity” means that the two different metals or metal alloys are either touching or in close enough proximity to each other such that when the two different metals are in contact with an electrolyte, the electrolyte becomes electrically conductive and ion migration occurs between one of the metals and the other metal, and is not meant to require an actual physical connection between the two different metals, for example, via a metal wire. It is to be understood that as used herein, the term “metal” is meant to include pure metals and also metal alloys without the need to continually specify that the metal can also be a metal alloy. Moreover, the use of the phrase “metal or metal alloy” in one sentence or paragraph does not mean that the mere use of the word “metal” in another sentence or paragraph is meant to exclude a metal alloy. As used herein, the term “metal alloy” means a mixture of two or more elements, wherein at least one of the elements is a metal. The other element(s) can be a non-metal or a different metal. An example of a metal and non-metal alloy is steel, comprising the metal element iron

and the non-metal element carbon. An example of a metal and metal alloy is bronze, comprising the metallic elements copper and tin.

The metal that is less noble, compared to the other metal, will dissolve in the electrolyte. The less noble metal is often referred to as the anode, and the more noble metal is often referred to as the cathode. Galvanic corrosion is an electrochemical process whereby free ions in the electrolyte make the electrolyte electrically conductive, thereby providing a means for ion migration from the anode to the cathode—resulting in deposition formed on the cathode. Metals can be arranged in a galvanic series. The galvanic series lists metals in order of the most noble to the least noble. An anodic index lists the electrochemical voltage (V) that develops between a metal and a standard reference electrode (gold (Au)) in a given electrolyte. The actual electrolyte used can affect where a particular metal or metal alloy appears on the galvanic series and can also affect the electrochemical voltage. For example, the dissolved oxygen content in the electrolyte can dictate where the metal or metal alloy appears on the galvanic series and the metal’s electrochemical voltage. The anodic index of gold is  $-0\text{ V}$ ; while the anodic index of beryllium is  $-1.85\text{ V}$ . A metal that has an anodic index greater than another metal is more noble than the other metal and will function as the cathode. Conversely, the metal that has an anodic index less than another metal is less noble and functions as the anode. In order to determine the relative voltage between two different metals, the anodic index of the lesser noble metal is subtracted from the other metal’s anodic index, resulting in a positive value.

There are several factors that can affect the rate of galvanic corrosion. One of the factors is the distance separating the metals on the galvanic series chart or the difference between the anodic indices of the metals. For example, beryllium is one of the last metals listed at the least noble end of the galvanic series and platinum is one of the first metals listed at the most noble end of the series. By contrast, tin is listed directly above lead on the galvanic series. Using the anodic index of metals, the difference between the anodic index of gold and beryllium is  $1.85\text{ V}$ ; whereas, the difference between tin and lead is  $0.05\text{ V}$ . This means that galvanic corrosion will occur at a much faster rate for magnesium or beryllium and gold compared to lead and tin.

The following is a partial galvanic series chart using a deoxygenated sodium chloride water solution as the electrolyte. The metals are listed in descending order from the most noble (cathodic) to the least noble (anodic). The following list is not exhaustive, and one of ordinary skill in the art is able to find where a specific metal or metal alloy is listed on a galvanic series in a given electrolyte.

---

|    |                                                    |
|----|----------------------------------------------------|
| 55 | PLATINUM                                           |
|    | GOLD                                               |
| 50 | ZIRCONIUM                                          |
|    | GRAPHITE                                           |
|    | SILVER                                             |
| 60 | CHROME IRON                                        |
|    | SILVER SOLDER                                      |
| 65 | COPPER-NICKEL ALLOY 80-20                          |
|    | COPPER-NICKEL ALLOY 90-10                          |
|    | MANGANESE BRONZE (CA 675), TIN BRONZE (CA903, 905) |
|    | COPPER (CA102)                                     |
|    | BRASSES                                            |
|    | NICKEL (ACTIVE)                                    |
|    | TIN                                                |
|    | LEAD                                               |
|    | ALUMINUM BRONZE                                    |
|    | STAINLESS STEEL                                    |

CHROME IRON  
MILD STEEL (1018), WROUGHT IRON  
ALUMINUM 2117, 2017, 2024  
CADMIUM  
ALUMINUM 5052, 3004, 3003, 1100, 6053  
ZINC  
MAGNESIUM  
BERYLLIUM

The following is a partial anodic index listing the voltage of a listed metal against a standard reference electrode (gold) using a deoxygenated sodium chloride water solution as the electrolyte. The metals are listed in descending order from the greatest voltage (most cathodic) to the least voltage (most anodic). The following list is not exhaustive, and one of ordinary skill in the art is able to find the anodic index of a specific metal or metal alloy in a given electrolyte.

the wellbore isolation device to come in contact with an electrolyte; and allowing at least a portion of the first material to dissolve.

Any discussion of the embodiments regarding the isolation device or any component related to the isolation device (e.g., the electrolyte) is intended to apply to all of the apparatus and method embodiments.

Turning to the Figures, FIG. 1 depicts a well system 10. The well system 10 can include at least one wellbore 11. The wellbore 11 can penetrate a subterranean formation 20. The subterranean formation 20 can be a portion of a reservoir or adjacent to a reservoir. The wellbore 11 can include a casing 12. The wellbore 11 can include only a generally vertical wellbore section or can include only a generally horizontal wellbore section. A first section of tubing string 15 can be installed in the wellbore 11. A second section of tubing string 16 (as well as multiple other sections of tubing string, not shown) can be installed in the wellbore 11. The well system

| Anodic index                                                                                                                     |           |
|----------------------------------------------------------------------------------------------------------------------------------|-----------|
| Metal                                                                                                                            | Index (V) |
| Gold, solid and plated, Gold-platinum alloy                                                                                      | -0.00     |
| Rhodium plated on silver-plated copper                                                                                           | -0.05     |
| Silver, solid or plated; monel metal. High nickel-copper alloys                                                                  | -0.15     |
| Nickel, solid or plated; titanium an s alloys, Monel                                                                             | -0.30     |
| Copper, solid or plated; low brasses or bronzes; silver solder; German silvery high copper-nickel alloys; nickel-chromium alloys | -0.35     |
| Brass and bronzes                                                                                                                | -0.40     |
| High brasses and bronzes                                                                                                         | -0.45     |
| 18% chromium type corrosion-resistant steels                                                                                     | -0.50     |
| Chromium plated; tin plated; 12% chromium type corrosion-resistant steels                                                        | -0.60     |
| Tin-plate; tin-lead solder                                                                                                       | -0.65     |
| Lead, solid or plated; high lead alloys                                                                                          | -0.70     |
| 2000 series wrought aluminum                                                                                                     | -0.75     |
| Iron, wrought, gray or malleable, plain carbon and low alloy steels                                                              | -0.85     |
| Aluminum, wrought alloys other than 2000 series aluminum, cast alloys of the silicon type                                        | -0.90     |
| Aluminum, cast alloys other than silicon type, cadmium, plated and chromate                                                      | -0.95     |
| Hot-dip-zinc plate; galvanized steel                                                                                             | -1.20     |
| Zinc, wrought; zinc-base die-casting alloys; zinc plated                                                                         | -1.25     |
| Magnesium & magnesium-base alloys, cast or wrought                                                                               | -1.75     |
| Beryllium                                                                                                                        | -1.85     |

Another factor that can affect the rate of galvanic corrosion is the temperature and concentration of the electrolyte. The higher the temperature and concentration of the electrolyte, the faster the rate of corrosion. Yet another factor that can affect the rate of galvanic corrosion is the total amount of surface area of the least noble (anodic metal). The greater the surface area of the anode that can come in contact with the electrolyte, the faster the rate of corrosion. The cross-sectional size of the anodic metal pieces can be decreased in order to increase the total amount of surface area per total volume of the material. Yet another factor that can affect the rate of galvanic corrosion is the ambient pressure. Depending on the electrolyte chemistry and the two metals, the corrosion rate can be slower at higher pressures than at lower pressures if gaseous components are generated.

According to an embodiment, a wellbore isolation device comprises: at least a first material, wherein the first material: (A) is a metal or a metal alloy; and (B) is capable of at least partially dissolving when an electrically conductive path exists between the first material and a second material and at least a portion of the first and second materials are in contact with an electrolyte, wherein the second material: (i) is a metal or metal alloy; and (ii) has a greater anodic index than the first material.

According to another embodiment, a method of removing a wellbore isolation device comprises: contacting or allowing

10 can comprise at least a first zone 13 and a second zone 14. The well system 10 can also include more than two zones, for example, the well system 10 can further include a third zone, a fourth zone, and so on. The well system 10 can further include one or more packers 18. The packers 18 can be used in addition to the isolation device to isolate each zone of the wellbore 11.

50 The isolation device can be the packers 18. The packers 18 can be used to prevent fluid flow between one or more zones (e.g., between the first zone 13 and the second zone 14) via an annulus 19. The tubing string 15/16 can also include one or more ports 17. One or more ports 17 can be located in each 55 section of the tubing string. Moreover, not every section of the tubing string needs to include one or more ports 17. For example, the first section of tubing string 15 can include one or more ports 17, while the second section of tubing string 16 does not contain a port. In this manner, fluid flow into the annulus 19 for a particular section can be selected based on the specific oil or gas operation.

It should be noted that the well system 10 is illustrated in the drawings and is described herein as merely one example of a wide variety of well systems in which the principles of this disclosure can be utilized. It should be clearly understood that the principles of this disclosure are not limited to any of the details of the well system 10, or components thereof,

depicted in the drawings or described herein. Furthermore, the well system 10 can include other components not depicted in the drawing. For example, the well system 10 can further include a well screen. By way of another example, cement may be used instead of packers 18 to aid the isolation device in providing zonal isolation. Cement may also be used in addition to packers 18.

According to an embodiment, the isolation device is capable of restricting or preventing fluid flow between a first zone 13 and a second zone 14. The first zone 13 can be located upstream or downstream of the second zone 14. In this manner, depending on the oil or gas operation, fluid is restricted or prevented from flowing downstream or upstream into the second zone 14. Examples of isolation devices capable of restricting or preventing fluid flow between zones include, but are not limited to, a ball and seat, a plug, a bridge plug, a wiper plug, and a packer.

Referring to FIGS. 2-4, the isolation device comprises at least a first material 51, wherein the first material is capable of at least partially dissolving when an electrically conductive path exists between the first material 51 and a second material 52. The first material 51 and the second material 52 are metals or metal alloys. The metal or metal alloy can be selected from the group consisting of, lithium, sodium, potassium, rubidium, cesium, francium, beryllium, magnesium, calcium, strontium, barium, radium, aluminum, gallium, indium, tin, thallium, lead, bismuth, scandium, titanium, vanadium, chromium, manganese, iron, cobalt, nickel, copper, zinc, yttrium, zirconium, niobium, molybdenum, technetium, ruthenium, rhodium, palladium, silver, cadmium, lanthanum, hafnium, tantalum, tungsten, rhenium, osmium, iridium, platinum, gold, graphite, and combinations thereof. Preferably, the metal or metal alloy is selected from the group consisting of beryllium, tin, iron, nickel, copper, zinc, and combinations thereof. According to an embodiment, the metal is neither radioactive, unstable, nor theoretical.

According to an embodiment, the first material 51 and the second material 52 are different metals or metal alloys. By way of example, the first material 51 can be nickel and the second material 52 can be gold. Furthermore, the first material 51 can be a metal and the second material 52 can be a metal alloy. The first material 51 and the second material 52 can be a metal and the first and second material can be a metal alloy. The second material 52 has a greater anodic index than the first material 51. Stated another way, the second material 52 is listed higher on a galvanic series than the first material 51. According to another embodiment, the second material 52 is more noble than the first material 51. In this manner, the first material 51 acts as an anode and the second material 52 acts as a cathode. Moreover, in this manner, the first material 51 (acting as the anode) at least partially dissolves when in electrical connectivity with the second material 52 and when the first and second materials are in contact with the electrolyte.

The methods include the step of allowing at least a portion of the first material to dissolve. The step of allowing at least a portion of the first material to dissolve can be performed after the step of contacting or allowing the first material to come in contact with the electrolyte. At least a portion of the first material 51 can dissolve in a desired amount of time. The desired amount of time can be pre-determined, based in part, on the specific oil or gas well operation to be performed. The desired amount of time can be in the range from about 1 hour to about 2 months. There are several factors that can affect the rate of dissolution of the first material 51. According to an embodiment, the first material 51 and the second material 52 are selected such that the at least a portion of the first material

51 dissolves in the desired amount of time. By way of example, the greater the difference between the second material's anodic index and the first material's anodic index, the faster the rate of dissolution. By contrast, the less the difference between the second material's anodic index and the first material's anodic index, the slower the rate of dissolution. By way of yet another example, the farther apart the first material and the second material are from each other in a galvanic series, the faster the rate of dissolution; and the closer together the first and second material are to each other in the galvanic series, the slower the rate of dissolution. By evaluating the difference in the anodic index of the first and second materials, or by evaluating the order in a galvanic series, one of ordinary skill in the art will be able to determine the rate of dissolution of the first material in a given electrolyte.

Another factor that can affect the rate of dissolution of the first material 51 is the proximity of the first material 51 to the second material 52. A more detailed discussion regarding different embodiments of the proximity of the first and second materials is presented below. Generally, the closer the first material 51 is physically to the second material 52, the faster the rate of dissolution of the first material 51. By contrast, generally, the farther apart the first and second materials are from one another, the slower the rate of dissolution. It should be noted that the distance between the first material 51 and the second material 52 should not be so great that an electrically conductive path ceases to exist between the first and second materials. According to an embodiment, any distance between the first and second materials 51/52 is selected such that the at least a portion of the first material 51 dissolves in the desired amount of time.

Another factor that can affect the rate of dissolution of the first material 51 is the concentration of the electrolyte and the temperature of the electrolyte. A more detailed discussion of the electrolyte is presented below. Generally, the higher the concentration of the electrolyte, the faster the rate of dissolution of the first material 51, and the lower the concentration of the electrolyte, the slower the rate of dissolution. Moreover, the higher the temperature of the electrolyte, the faster the rate of dissolution of the first material 51, and the lower the temperature of the electrolyte, the slower the rate of dissolution. One of ordinary skill in the art can select: the exact metals and/or metal alloys, the proximity of the first and second materials, and the concentration of the electrolyte based on an anticipated temperature in order for the at least a portion of the first material 51 to dissolve in the desired amount of time.

As can be seen in FIG. 1, the first section of tubing string 15 can be located within the first zone 13 and the second section of tubing string 16 can be located within the second zone 14. 50 As depicted in the drawings, the isolation device can be a ball 30 (e.g., a first ball 31 or a second ball 32) and a seat 40 (e.g., a first seat 41 or a second seat 42). The ball 30 can engage the seat 40. The seat 40 can be located on the inside of a tubing string. When the first section of tubing string 15 is located downstream of the second section of tubing string 16, then the inner diameter (I.D.) of the first section of tubing string 15 can be less than the I.D. of the second section of tubing string 16. In this manner, a first ball 31 can be placed into the first section of tubing string 15. The first ball 31 can have a smaller diameter than a second ball 32. The first ball 31 can engage a first seat 41. Fluid can now be temporarily restricted or prevented from flowing into any zones located downstream of the first zone 13. In the event it is desirable to temporarily restrict or prevent fluid flow into any zones located downstream of the second zone 14, the second ball 32 can be placed into second section of tubing string 16 and will be prevented from falling into the first section of tubing string 15 via the

second seat 42 or because the second ball 32 has a larger outer diameter (O.D.) than the I.D. of the first section of tubing string 15. The second ball 32 can engage the second seat 42. The ball (whether it be a first ball 31 or a second ball 32) can engage a sliding sleeve 33 during placement. This engagement with the sliding sleeve 33 can cause the sliding sleeve to move; thus, opening a port 17 located adjacent to the seat. The port 17 can also be opened via a variety of other mechanisms instead of a ball. The use of other mechanisms may be advantageous when the isolation device is not a ball. After placement of the isolation device, fluid can be flowed from, or into, the subterranean formation 20 via one or more opened ports 17 located within a particular zone. As such, a fluid can be produced from the subterranean formation 20 or injected into the formation.

FIGS. 2-4 depict the isolation device according to certain embodiments. As can be seen in the drawings, the isolation device can be a ball 30. As depicted in FIG. 2, the isolation device can comprise the first material 51 and the second material 52. According to this embodiment, the first and second materials 51/52 can be nuggets of material. Although this embodiment depicted in FIG. 2 illustrates the isolation device as a ball, it is to be understood that this embodiment and discussion thereof is equally applicable to an isolation device that is a bridge plug, packer, etc. The nuggets of the first material 51 and the nuggets of the second material 52 can be bonded together in a variety of ways in order to form the isolation device. At least a portion of the outside of the nuggets of the first material 51 can be in direct contact with at least a portion of the outside of the nuggets of the second material 52. By contrast, the outside of the nuggets of the first material 51 do not have to be in direct contact with the outside of the nuggets of the second material 52. For example, there can be an intermediary substance located between the outside of the nuggets of the first and second materials 51/52. The intermediary substance can be, without limitation, another metal or metal alloy, a non-metal, a plastic, or sand. In order for galvanic corrosion to occur (and hence dissolution of at least a portion of the first material 51), both, the first and second materials 51/52 need to be capable of being contacted by the electrolyte. Preferably, at least a portion of one or more nugget of the first material 51 and the second material 52 form the outside of the isolation device, such as a ball 30. In this manner, at least a portion of the first and second materials 51/52 are capable of being contacted with the electrolyte.

The size, shape and placement of the nuggets of the first and second materials 51/52 can be adjusted to control the rate of dissolution of the first material 51. By way of example, generally the smaller the cross-sectional area of each nugget, the faster the rate of dissolution. The smaller cross-sectional area increases the ratio of the surface area to total volume of the material, thus allowing more of the material to come in contact with the electrolyte. The cross-sectional area of each nugget of the first material 51 can be the same or different, the cross-sectional area of each nugget of the second material 52 can be the same or different, and the cross-sectional area of the nuggets of the first material 51 and the nuggets of the second material 52 can be the same or different. Additionally, the cross-sectional area of the nuggets forming the outer portion of the isolation device and the nuggets forming the inner portion of the isolation device can be the same or different. By way of example, if it is desired for the outer portion of the isolation device to proceed at a faster rate of galvanic corrosion compared to the inner portion of the device, then the cross-sectional area of the individual nuggets comprising the outer portion can be smaller compared to the cross-sectional area of the nuggets comprising the inner portion. The shape of

the nuggets of the first and second materials 51/52 can also be adjusted to allow for a greater or smaller cross-sectional area. The proximity of the first material 51 to the second material 52 can also be adjusted to control the rate of dissolution of the first material 51. According to an embodiment, the first and second materials 51/52 are within 2 inches, preferably less than 1 inch of each other.

FIGS. 3 and 4 depict the isolation device according to other embodiments. As can be seen in FIG. 3, the isolation device, 10 such as a ball 30, can be made entirely of the first material 51. As can be seen in FIG. 4, the isolation device, such as a ball 30, can comprise the first material 51. The isolation device illustrated in FIG. 4 can include an outer layer of the first material 51. The thickness  $t$  of the outer layer can be adjusted 15 to control the rate of dissolution of the first material 51. The isolation device shown in FIG. 4 can also include a substance 60 forming the inside of the isolation device. The inside can also be hollow. The substance 60 can be, without limitation, a non-metal, a plastic, or sand. Preferably, the substance 60 is 20 selected and has a cross-sectional area such that after dissolution of the first material 51, the isolation device is capable of being flowed from the wellbore 11. By way of example, if the substance 60 is sand, then the sand is capable of being flowed from the wellbore without needing to adjust the size of the sand. By contrast, if the substance 60 is a plastic, then the cross-sectional area of the plastic might need to be adjusted 25 such that the isolation device is capable of being flowed from the wellbore 11.

As shown in FIGS. 3 and 4, at least a portion of a seat 40 can 30 comprise the second material 52. According to this embodiment, at least a portion of the first material 51 of the ball 30 can come in contact with at least a portion of the second material 52 of the seat 40. Although not shown in the drawings, according to another embodiment, at least a portion of a 35 tubing string can comprise the second material 52. This embodiment can be useful for a ball, bridge plug, packer, etc. isolation device. Preferably, the portion of the tubing string that comprises the second material 52 is located adjacent to the isolation device comprising the first material 51. More 40 preferably, the portion of the tubing string that comprises the second material 52 is located adjacent to the isolation device comprising the first material 51 after the isolation device is situated in the desired location within the wellbore 11. The portion of the tubing string that comprises the second material 45 52 is preferably located within a maximum distance to the isolation device comprising the first material 51. The maximum distance can be a distance such that an electrically conductive path exists between the first material 51 and the second material 52. In this manner, once the isolation device is situated within the wellbore 11 and the first and second materials 51/52 are in contact with the electrolyte, at least a portion of the first material 51 is capable of dissolving due to the electrical connectivity between the materials.

According to an embodiment, at least the first material 51 55 is capable of withstanding a specific pressure differential (for example, the isolation device depicted in FIG. 3). As used herein, the term "withstanding" means that the substance does not crack, break, or collapse. The pressure differential can be the downhole pressure of the subterranean formation 20 across the device. As used herein, the term "downhole" means the location of the wellbore where the first material 51 is located. Formation pressures can range from about 1,000 to about 30,000 pounds force per square inch (psi) (about 6.9 to about 206.8 megapascals ("MPa"). The pressure differential 60 can also be created during oil or gas operations. For example, a fluid, when introduced into the wellbore 11 upstream or downstream of the substance, can create a higher pressure

## 11

above or below, respectively, of the isolation device. Pressure differentials can range from 100 to over 10,000 psi (about 0.7 to over 68.9 MPa). According to another embodiment, both, the first and second materials **51/52** are capable of withstanding a specific pressure differential (for example, the isolation device depicted in FIG. 2). According to yet another embodiment, both, the first material **51** and the substance **60** are capable of withstanding a specific pressure differential (for example, the isolation device depicted in FIG. 4). The isolation device can also include a hollow core without the substance **60**. According to this embodiment, the first material **51** is capable of withstanding a specific pressure differential.

As discussed above, the rate of dissolution of the first material **51** can be controlled using a variety of factors. According to an embodiment, at least the first material **51** includes one or more tracers (not shown). The tracer(s) can be, without limitation, radioactive, chemical, electronic, or acoustic. The second material **52** and/or the substance **60** can also include one or more tracers. As depicted in FIG. 2, each nugget of the first material **51** can include a tracer. As depicted in FIG. 3, at least one tracer can be located near the outside of the isolation device and/or at least one tracer can be located near the inside of the device. Moreover, at least one tracer can be located in multiple layers of the device. As depicted in FIG. 4, at least one tracer can be located in the first material **51** and/or at least one tracer can be located in the substance **60**. A tracer can be useful in determining real-time information on the rate of dissolution of the first material **51**. For example, a first material **51** containing a tracer, upon dissolution can be flowed through the wellbore **11** and towards the wellhead or into the subterranean formation **20**. By being able to monitor the presence of the tracer, workers at the surface can make on-the-fly decisions that can affect the rate of dissolution of the remaining first material **51**.

Such decisions might include to increase or decrease the concentration of the electrolyte. As used herein, an electrolyte is any substance containing free ions (i.e., a positive- or negative-electrically charged atom or group of atoms) that make the substance electrically conductive. The electrolyte can be selected from the group consisting of, solutions of an acid, a base, a salt, and combinations thereof. A salt can be dissolved in water, for example, to create a salt solution. Common free ions in an electrolyte include sodium ( $\text{Na}^+$ ), potassium ( $\text{K}^+$ ), calcium ( $\text{Ca}^{2+}$ ), magnesium ( $\text{Mg}^{2+}$ ), chloride ( $\text{Cl}^-$ ), hydrogen phosphate ( $\text{HPO}_4^{2-}$ ), and hydrogen carbonate ( $\text{HCO}_3^-$ ). The concentration (i.e., the total number of free ions available in the electrolyte) of the electrolyte can be adjusted to control the rate of dissolution of the first material **51**. According to an embodiment, the concentration of the electrolyte is selected such that the at least a portion of the first material **51** dissolves in the desired amount of time. If more than one electrolyte is used, then the concentration of the electrolytes is selected such that the first material **51** dissolves in a desired amount of time. The concentration can be determined based on at least the specific metals or metal alloys selected for the first and second materials **51/52** and the bottomhole temperature of the well. Moreover, because the free ions in the electrolyte enable the electrochemical reaction to occur between the first and second materials **51/52** by donating its free ions, the number of free ions will decrease as the reaction occurs. At some point, the electrolyte may be depleted of free ions if there is any remaining first and second materials **51/52** that have not reacted. If this occurs, the galvanic corrosion that causes the first material **51** to dissolve will stop. In this example, it may be necessary to cause or allow the first and second materials to come in contact with a second, third, or fourth, and so on, electrolyte(s).

## 12

The methods include the step of contacting or allowing the wellbore isolation device to come in contact with the electrolyte. The step of contacting can include introducing the electrolyte into the wellbore **11**. The step of allowing can include 5 allowing the isolation device to come in contact with a fluid, such as a reservoir fluid. The methods can include contacting or allowing the device to come in contact with two or more electrolytes. If more than one electrolyte is used, the free ions in each electrolyte can be the same or different. A first electrolyte can be, for example, a stronger electrolyte compared to a second electrolyte. Furthermore, the concentration of each electrolyte can be the same or different. It is to be understood 10 that when discussing the concentration of an electrolyte, it is meant to be a concentration prior to contact with either the first and second materials **51/52**, as the concentration will decrease during the galvanic corrosion reaction. Tracers can be used to help determine the necessary concentration of the electrolyte to help control the rate and finality of dissolution of the first material **51**. For example, if it is desired that the 15 first material **51** dissolves to a point to enable the isolation device to be flowed from the wellbore **11** within 5 days and information from a tracer indicates that the rate of dissolution is too slow, then a more concentrated electrolyte can be introduced into the wellbore or allowed to contact the first and 20 second materials **51/52**. By contrast, if the rate of dissolution is occurring too quickly, then the first electrolyte can be flushed from the wellbore and a less concentrated electrolyte 25 can then be introduced into the wellbore.

It may be desirable to delay contact of at least the first 30 material **51** with the electrolyte. The isolation device can further include a coating on the outside of the device. The coating can be a compound, such as a wax, thermoplastic, sugar, salt, or polymer. The coating can be selected such that the coating either dissolves in wellbore fluids or melts at a 35 certain temperature. Upon dissolution or melting, at least the first material **51** of the isolation device is available to come in contact with the electrolyte. It may also be desirable to selectively dissolve certain portions of the first material **51** at different times or at different rates. By way of example, it may 40 be desirable to dissolve the top portion of the isolation device first and then dissolve the bottom portion at a later time. This can be accomplished, for example, by introducing a first electrolyte into the wellbore to come in contact with the first and second materials **51/52**. There are many operations, such 45 as stimulation operations involving fracturing or acidizing techniques, or tertiary recovery operations involving injection techniques, in which this may be desirable. After the desired operation has been performed, the bottom of the isolation device can be contacted by produced formation 50 fluids. The formation fluids can contain a sufficient concentration of free ions to allow the dissolution of the remaining first material **51**.

The methods can further include the step of placing the 55 isolation device in a portion of the wellbore **11**, wherein the step of placing is performed prior to the step of contacting or allowing the isolation device to come in contact with the electrolyte. More than one isolation device can also be placed in multiple portions of the wellbore. The methods can further include the step of removing all or a portion of the dissolved first material **51** and/or all or a portion of the second material **52** or the substance **60**, wherein the step of removing is 60 performed after the step of allowing the at least a portion of the first material to dissolve. The step of removing can include flowing the dissolved first material **51** and/or the second material **52** or substance **60** from the wellbore **11**. According to an embodiment, a sufficient amount of the first material **51** dissolves such that the isolation device is capable of being

## 13

flowed from the wellbore 11. According to this embodiment, the isolation device should be capable of being flowed from the wellbore via dissolution of the first material 51, without the use of a milling apparatus, retrieval apparatus, or other such apparatus commonly used to remove isolation devices. According to an embodiment, after dissolution of the first material 51, the second material 52 or the substance 60 has a cross-sectional area less than 0.05 square inches, preferably less than 0.01 square inches.

Therefore, the present invention is well adapted to attain the ends and advantages mentioned as well as those that are inherent therein. The particular embodiments disclosed above are illustrative only, as the present invention may be modified and practiced in different but equivalent manners apparent to those skilled in the art having the benefit of the teachings herein. Furthermore, no limitations are intended to the details of construction or design herein shown, other than as described in the claims below. It is, therefore, evident that the particular illustrative embodiments disclosed above may be altered or modified and all such variations are considered within the scope and spirit of the present invention. While compositions and methods are described in terms of "comprising," "containing," or "including" various components or steps, the compositions and methods also can "consist essentially of" or "consist of" the various components and steps. Whenever a numerical range with a lower limit and an upper limit is disclosed, any number and any included range falling within the range is specifically disclosed. In particular, every range of values (of the form, "from about a to about b," or, equivalently, "from approximately a to b") disclosed herein is to be understood to set forth every number and range encompassed within the broader range of values. Also, the terms in the claims have their plain, ordinary meaning unless otherwise explicitly and clearly defined by the patentee. Moreover, the indefinite articles "a" or "an", as used in the claims, are defined herein to mean one or more than one of the element that it introduces. If there is any conflict in the usages of a word or term in this specification and one or more patent(s) or other documents that may be incorporated herein by reference, the definitions that are consistent with this specification should be adopted.

What is claimed is:

1. A method of removing a wellbore isolation device comprising:  
 45 contacting or allowing the wellbore isolation device to come in contact with an electrolyte, wherein the wellbore isolation device comprises:  
 (A) a first material, wherein the first material:  
 50 (i) is a metal or a metal alloy; and  
 (ii) is capable of at least partially dissolving when an electrically conductive path exists between the first material and a second material and at least a portion of the first and second materials are in contact with the electrolyte; and  
 (B) the second material, wherein the second material:  
 55 (i) is a metal or metal alloy; and  
 (ii) has a greater anodic index than the first material, wherein the first material and the second material are nuggets; and  
 allowing at least a portion of the first material to dissolve, wherein the at least a portion of the first material dissolves in a desired amount of time,  
 60 wherein any distance between the first and second materials is selected such that the at least a portion of the first material dissolves in the desired amount of time.

## 14

2. The method according to claim 1, wherein the isolation device is capable of restricting or preventing fluid flow between a first zone and a second zone of the wellbore.  
 5 3. The method according to claim 1, wherein isolation device is a ball and a seat, a plug, a bridge plug, a wiper plug, or a packer.  
 4. The method according to claim 1, wherein the metal or metal alloy of the first material and the second material are selected from the group consisting of, beryllium, tin, iron, nickel, copper, zinc, graphite, and combinations thereof.  
 10 5. The method according to claim 1, wherein the metals or metal alloys of the first material and the second material are selected such that the at least a portion of the first material dissolves in the desired amount of time.  
 15 6. The method according to claim 1, wherein the concentration of the electrolyte is selected such that the at least a portion of the first material dissolves in the desired amount of time.  
 7. The method according to claim 1, wherein at least a 20 portion of one or more nuggets of the first material and one or more nuggets of the second material form the outside of the isolation device.  
 25 8. The method according to claim 1, wherein at least the first material is capable of withstanding a specific pressure differential.  
 9. The method according to claim 8, wherein the pressure differential is in the range from about 100 to about 25,000 pounds force per square inch (psi) (about 0.7 to about 172.4 megapascals).  
 30 10. The method according to claim 1, wherein the wellbore isolation device further comprises one or more tracers.  
 11. The method according to claim 1, wherein the step of contacting can include introducing an electrolyte into the wellbore.  
 35 12. The method according to claim 1, further comprising the step of placing the isolation device into a portion of the wellbore, wherein the step of placing is performed prior to the step of contacting or allowing the isolation device to come in contact with the electrolyte.  
 40 13. The method according to claim 1, further comprising the step of removing all or a portion of the dissolved first material, wherein the step of removing is performed after the step of allowing the at least a portion of the first material to dissolve.  
 14. A wellbore isolation device comprising:  
 a first material, wherein the first material:  
 (A) is a metal or a metal alloy; and  
 45 (B) is capable of at least partially dissolving when an electrically conductive path exists between the first material and a second material and at least a portion of the first and second materials are in contact with an electrolyte; and  
 the second material, wherein the second material:  
 (A) is a metal or metal alloy; and  
 (B) has a greater anodic index than the first material, wherein the first material and the second material are nuggets,  
 50 wherein at least a portion of the first material dissolves in a desired amount of time, and  
 wherein any distance between the first and second materials is selected such that the at least a portion of the first material dissolves in the desired amount of time.  
 55 15. A method of removing a wellbore isolation device comprising:  
 contacting or allowing the wellbore isolation device to come in contact with an electrolyte, wherein the wellbore isolation device comprises:

**15**

at least a first material, wherein the first material:

- is a metal or a metal alloy; and
- is capable of at least partially dissolving when an electrically conductive path exists between the first material and a second material and at least a portion of the first and second materials are in contact with the electrolyte,

wherein the isolation device comprises an outer layer of the first material, and

wherein the second material:

- is a metal or metal alloy; and
- has a greater anodic index than the first material; and

allowing at least a portion of the first material to dissolve, wherein the at least a portion of the first material dissolves in a desired amount of time, and

wherein any distance between the first and second materials is selected such that the at least a portion of the first material dissolves in the desired amount of time.

**16.** The method according to claim **15**, wherein the isolation device further comprises a substance forming the inside of the isolation device.

**17.** The method according to claim **16**, wherein the substance is selected from the group consisting of a metal or metal alloy, a non-metal, a plastic, sand, and combinations thereof.

**18.** The method according to claim **16**, further comprising the step of removing all or a portion of the dissolved first material and the second material or the substance, wherein the step of removing is performed after the step of allowing the at least a portion of the first material to dissolve.

**19.** A method of removing a wellbore isolation device comprising:

contacting or allowing the wellbore isolation device to come in contact with an electrolyte, wherein the wellbore isolation device comprises:

at least a first material, wherein the first material:

- is a metal or a metal alloy; and
- is capable of at least partially dissolving when an electrically conductive path exists between the first material and a second material and at least a portion of the first and second materials are in contact with the electrolyte,

wherein the second material:

- is a metal or metal alloy; and
- has a greater anodic index than the first material, and

5

10

15

20

25

30

35

40

45

45

**16**

wherein the isolation device is a ball and at least a portion of a seat comprises the second material; and allowing at least a portion of the first material to dissolve, wherein the at least a portion of the first material dissolves in a desired amount of time, and

wherein any distance between the first and second materials is selected such that the at least a portion of the first material dissolves in the desired amount of time.

**20.** A wellbore isolation device comprising:

at least a first material, wherein the first material:

- is a metal or a metal alloy; and
- is capable of at least partially dissolving when an electrically conductive path exists between the first material and a second material and at least a portion of the first and second materials are in contact with an electrolyte,

wherein the isolation device comprises an outer layer of the first material,

wherein the second material:

- is a metal or metal alloy; and
- has a greater anodic index than the first material, wherein at least a portion of the first material dissolves in a desired amount of time, and

wherein any distance between the first and second materials is selected such that the at least a portion of the first material dissolves in the desired amount of time.

**21.** A wellbore isolation device comprising:

at least a first material, wherein the first material:

- is a metal or a metal alloy; and
- is capable of at least partially dissolving when an electrically conductive path exists between the first material and a second material and at least a portion of the first and second materials are in contact with an electrolyte,

wherein the second material:

- is a metal or metal alloy; and
- has a greater anodic index than the first material, wherein the isolation device is a ball and at least a portion of a seat comprises the second material, wherein at least a portion of the first material dissolves in a desired amount of time, and

wherein any distance between the first and second materials is selected such that the at least a portion of the first material dissolves in the desired amount of time.

\* \* \* \* \*

UNITED STATES PATENT AND TRADEMARK OFFICE  
**CERTIFICATE OF CORRECTION**

PATENT NO. : 8,905,147 B2  
APPLICATION NO. : 13/491995  
DATED : December 9, 2014  
INVENTOR(S) : Syed Hamid, Michael L. Fripp and Pete Dagenais

Page 1 of 1

It is certified that error appears in the above-identified patent and that said Letters Patent is hereby corrected as shown below:

Title Page, item (12), "Fripp et al." should read -- Hamid et al. --.

Title page, item (75), Inventors:, Cancel "Michael Fripp, Carrollton, TX (US)" and insert thereof  
-- Syed HAMID, Carrollton, TX (US) -- for the first named inventor; Cancel "Syed HAMID,  
Carrollton, TX (US)" and insert thereof -- Michael Fripp, Carrollton, TX (US) -- for the second named  
inventor.

In the Claims

Claim 3, column 14, line 4: "isolation" should be changed to -- the isolation --.

Signed and Sealed this  
Fourteenth Day of April, 2015



Michelle K. Lee  
*Director of the United States Patent and Trademark Office*